

# United States Patent [19]

Shinomiya et al.

[11] 3,930,081

[45] Dec. 30, 1975

[54] COMPOSITION AND PROCESS FOR  
DISPLACEMENT PLATING OF ZINC  
SURFACES

[75] Inventors: **Hiroshi Shinomiya**, Yokohama;  
**Kajuro Muro**, Komae; **Sumio Sakata**, Kobe; **Shigeki Saida**, Tokyo;  
**Seichiro Umehara**, Tokyo; **Yutaka Tsuchiya**, Tokyo; **Kunijo Yashiro**;  
**Yoshio Moriya**, both of Yokohama,  
all of Japan

[73] Assignee: **Oxy Metal Industries Corporation**,  
Warren, Mich.

[22] Filed: **Nov. 2, 1973**

[21] Appl. No.: **412,120**

## [30] Foreign Application Priority Data

Nov. 6, 1972 Japan ..... 47-110257  
Jan. 11, 1973 Japan ..... 48-5519

[52] U.S. Cl. ..... **427/421**; 106/1; 427/328;  
427/383; 427/405; 427/436

[51] Int. Cl.<sup>2</sup> ..... **C23C 3/00**

[58] Field of Search ..... 106/1; 148/6.14 R;  
117/130 R, 50; 427/436, 421, 328, 383, 405

## [56] References Cited

### UNITED STATES PATENTS

2,924,534 2/1960 Morse ..... 117/130 R X

|           |         |                    |             |
|-----------|---------|--------------------|-------------|
| 3,202,529 | 8/1965  | Dunlap .....       | 117/50 X    |
| 3,444,007 | 5/1969  | Maurer et al. .... | 148/6.14 X  |
| 3,468,724 | 9/1969  | Reinhold.....      | 117/130 R X |
| 3,539,403 | 11/1970 | Ries .....         | 148/6.14    |
| 3,672,964 | 6/1972  | Bellis .....       | 117/50 X    |

## OTHER PUBLICATIONS

Saubestre, "Electroless Plating Today", Aug. 1962,  
pp. 46-48.

Primary Examiner—Ralph S. Kendall

Assistant Examiner—John D. Smith

Attorney, Agent, or Firm—Arthur E. Kluegel; Richard  
P. Mueller; Bertram F. Claeboe

## [57] ABSTRACT

Disclosed is an improved composition and process for the heavy metal displacement plating of a zinc surface. The improved process provides for contacting the zinc surface with a solution containing at least one soluble stabilizing compound containing antimony, tin, copper, lead, germanium, vanadium, arsenic or tungsten. This contact may be effected either by pretreating the metal surface prior to displacement plating or by including the stabilizing compound in the displacement solution itself. The composition is an aqueous one containing both a heavy metal ion and the stabilizing compound. The disclosed process improves the displacement plating composition's resistance to degradation and consequent loss of efficiency.

2 Claims, No Drawings

**COMPOSITION AND PROCESS FOR  
DISPLACEMENT PLATING OF ZINC SURFACES**

**BACKGROUND OF THE INVENTION**

This invention relates to a composition and process for forming a coating on the surface of zinc or alloy thereof by contacting said surface with an acidic solution for displacement plating. It is an object of this invention to render such solutions less sensitive to zinc ion content thereby prolonging their useful life and improving the process efficiency. It is another object of this invention to provide an undercoating for paint having excellent adhesion characteristics.

Conventional processes for treating the surface of zinc or its alloys include displacement plating, chemical plating and chemical conversion coating processes such as chromating and sulfiding with black sulfides. The undercoatings produced by these conventional techniques have not been entirely satisfactory from the standpoint of corrosion and heat resistance or adhesion characteristics. Further in the acidic displacement plating processes, zinc ions are produced by the treated surface which gradually contaminate the solution, and thus, the initial efficiency for the plating cannot be maintained for a long period of time unless the spent solution is discarded and a fresh solution is supplied. Noticeable degradation of product quality occurs at zinc ion concentrations of 5 g/l and lower. It has now been found that a desensitized acidic solution for displacement plating containing nickel, iron or cobalt, suitable for forming a coating on the surface of zinc or an alloy thereof may be obtained by adding to the solution one or more soluble compounds of a desensitizing metal selected from antimony, tin, copper, lead, germanium, vanadium, arsenic and tungsten. It has also been found that the displacement solution may be rendered less sensitive to zinc ion content by contacting the zinc surface with a solution of one of the foregoing metals simultaneously with or prior to the displacement plating. Accordingly, this invention includes an acidic solution for the displacement plating in which a solution containing ionic nickel, iron, or cobalt, is adjusted to the desired pH by adding inorganic and/or organic acids and including a desensitizing metal compound and, if desired, a complexing agent. According to the method, the desensitizing metal compound may alternatively be employed in a pre-displacement plating treatment. Suitable heavy metal compounds of nickel, cobalt, and iron include the inorganic chlorides, sulfates, nitrates and carbonates and organic salts such as the acetates and citrates. Normally, the compound of heavy metal is contained in an amount more than 0.1 g/l, preferably in the range of from 0.1 to 50 g/l calculated as the metal.

Suitable desensitizing metal compounds include stannous chloride, tin borofluoride, stannous acetate, cupric chloride, cupric sulfate, copper citrate, lead chloride, lead nitrate, lead acetate, germanium chloride, germanium oxide, ammonium metavanadate, sodium arsenate, sodium hydrogen arsenate, ammonium magnesium arsenate, ammonium tungstate, sodium tungstate, potassium tungstate, potassium antimony tartrate, potassium antimony oxalate, sodium tetrachloro antimonate and antimony chloride. Such compounds are added to the pretreating solution or the solution for displacement plating in a total amount ranging from 0.001 to 50 g/l calculated as the metal and desirably

between 0.01 and 10 g/l. Since no effect can be achieved in an amount less than 0.001 g/l, and no proportional increase can be expected in the efficiency correspondingly to an amount more than 50 g/l, such amounts are economically disadvantageous. When the compounds are to be added to a pretreating solution, they may conveniently be added to the immediately preceding rinsing step or the pickling step.

Supplemental additives for the displacement solution include buffering compounds and a complexing agent for the metallic ions present in the solution or formed by the dissolution. These compounds include tartaric, citric, malic, oxalic, succinic acids and the like and the salts thereof. The amount to be added cannot be standardized depending on the purpose, but generally they are used in an amount ranging from 0.1 to 50 g/l.

In order to adjust the displacement plating solution to a desired pH value, organic or inorganic acids may be used. The inorganic acids include, for example, hydrochloric, sulfuric, hydrofluoric, and fluorosilicic, and the organic acids include citric, acetic, and oxalic. Normally, the acid will be present in an amount ranging from 1 to 150 g/l. If the desired pH can be obtained, a salt of such inorganic or organic acids may be used. For example, salts of a heavy metal such as iron, nickel, or cobalt, may be used.

The pH of the solution is generally maintained at a value less than 7 and preferably 1 to 4.5. The process of this invention comprises contacting the surface of zinc or an alloy thereof at a temperature ranging from room temperature to the boiling point of the solution for a sufficient length of time to obtain the desired coating by means of spraying, immersing or brushing, preferably by immersing or spraying for the case where the coating is to be used as an undercoating for painting. In a continuous process for forming a coating in a short period of time, it is desirable to treat the article with the solution at a temperature from 40° to 90°C for 2 to 6 seconds. While a satisfactory coating for use as an undercoating for paint can be obtained at a treating temperature of from 50° to 80°C for 3-30 seconds, it can be obtained in a shorter period of time with a higher concentration of the metallic ion and at higher treating temperatures. It takes somewhat longer time for the immersing process than that for the spraying process, but if an auxiliary means is adopted for stirring the solution or causing it to flow, the coating time is almost the same as that for the spraying process.

The coating treatment of this invention may be best effected by combining it with certain pretreating steps and after treating steps. The pretreating steps comprise steps for degreasing, etching by an acid or alkali solution, surface conditioning, and washing with water subsequent to each treating step. The degreasing step is employed when articles to be surface treated are processed in the presence of oil. The pickling step activates the surface of articles to be treated and strengthens the effect achieved by the main plating treatment. As an after treatment, it is preferable to rinse the formed coating with a dilute aqueous solution of chromic acid. The coating may then be rinsed with water and followed by drying. The coating then is ready for applying paints or other overcoatings. Both the pretreatments and after treatments referred to hereinbefore are normally effected for several seconds to 30 seconds.

The process of this invention is adapted for surfaces of zinc or its alloys including electrogalvanized and

hot-dip galvanized steel. By virtue of the treatment with a desensitizing metal compound, it is possible to maintain the initial efficiency for extended periods by inhibiting the deleterious effects normally caused by the increase in the amount of zinc ion dissolved in the plating solution. The coating obtained according to this invention has an excellent adhesion with paints as compared with phosphate coatings, complex coatings based on oxides and chromating coatings.

This invention will be further illustrated by means of the following examples.

### EXAMPLE 1 to 3

The adhesion of a film on galvanized steel after having been treated with the acidic solution for displacement plating according to this invention was compared with the film obtained from a conventional acidic solution for displacement plating. Specimens were samples from non-chromating galvanized steel plate (0.27 x 50 x 100 mm) having a zinc content of 183 grams/m<sup>2</sup>. The specimens were treated in a weak alkaline degreasing agent ("Finecleaner", Type 315 prepared by Nihon Parkerizing Co., Ltd.) in a concentration of 20 g/l at 60°C for 10 seconds and any trace of the residual degreasing agent was removed by rinsing with water. Then the specimens were pickled in 5% hydrochloric acid at 25°C for 5 seconds followed by rinsing with water again. The thus treated specimens were then subjected to displacement for plating using the compositions indicated at 60°C for 5 seconds. Then, the specimens were treated in a dilute chromic acid ("Percolene" Type 62 prepared by Nihon Parkerizing Co. Ltd.) in a concentration of 20 g/l, followed by removing excess chromic acid solution by squeezing them between rolls and finally drying by means of hot air at 105°C. The treatments were all effected by immersion.

#### Composition of the Displacement Plating Solution

The solution was prepared by dissolving nickel carbonate (16 grams), hydrochloric acid (35% : 30 grams), hydrofluoric acid (55% : 3 grams) and citric acid (5 grams) in city water 1 liter. Since the solution was reused repeatedly after the preparation, the components were constantly replenished in order to maintain the composition constant. Zinc was gradually dissolved into the solution from the surface treated and eventually reached a concentration of about 50 g/l. All of the examples and controls contained 65 g/l chloride, 1.6 g/l fluoride, 5 g/l citric acid and were adjusted to a pH of 2. In separate tests, desensitizing metal compounds were added as follows: sodium hydrogen arsenate (2.1 g/l); stannous chloride (0.96 g/l); germanium chloride (1.5 g/l). The compositions are summarized in Table I, excluding the Cl, F and Citric acid.

TABLE I

| Composition<br>Example | Ni <sup>2+</sup> | Zn <sup>2+</sup>  | As <sup>5+</sup>   | Sn <sup>2+</sup> | Ge <sup>4+</sup> | 2-T Bend |
|------------------------|------------------|-------------------|--------------------|------------------|------------------|----------|
| 1                      | 8 <sup>g/l</sup> | 50 <sup>g/l</sup> | 0.5 <sup>g/l</sup> | — <sup>g/l</sup> | — <sup>g/l</sup> | 4        |
| 2                      | 8                | 50                | —                  | 0.5              | —                | 4        |
| 3                      | 8                | 50                | —                  | —                | 0.5              | 3.4      |
| Control No. 1          | 8                | —                 | —                  | —                | —                | 4.2      |
| Control No. 2          | 8                | 50                | —                  | —                | —                | 1.0      |

The surface treated specimens were then coated with a polyester paint to a thickness of 12 microns and baked at 275°C for 90 seconds. Table I also shows the

results of adhesion test on the coated film effected after the baking.

Control specimens were also prepared from the same hot galvanized steel plate, plated with nickel, painted under the same conditions except that the solution contained no zinc ion in Control No. 1 and no arsenic nor stannous nor germanium ion in Control No. 2 and the adhesion of the coated film was tested. Table I shows also results of these controls.

#### Testing Procedure for the Adhesion of Coated Paint Film on the Metallic Surface (Bending Test)

After the coating of paint, the specimens were allowed to stand at 25°C for 24 hours. They were then folded 180°. The folded portion was pressed by means of a vise. Scotch tape was applied to the folded surface and was peeled off quickly after 1 minute from the application.

After the test, the specimens were evaluated according to the percentage of peeled area on the folded surface. When the specimens were pressed together by means of the vise, the testing condition can be modified from the severe to moderate ones by inserting a desired number of plates having the same thickness as that of specimens between the confronted surfaces of folded specimens. Corresponding to the number of plates inserted therebetween, the test results were designated as 1 T when one plate thickness was inserted, as 2 T when two plates were inserted and as 0 T when no plate was inserted therebetween. Accordingly, the smaller the number of the inserted plates was, the more severe the test condition becomes. Each test was repeated for 5 specimens and the average is reported.

The results were then classified in accordance with the following scale:

- 5 — No peeling or cracking of the film.
- 4 — Less than 1% peel.
- 3 — 2-25% peel.
- 2 — 26-50% peel.
- 1 — In excess of 50% peel.

#### EXAMPLES 4 to 6

Additional specimens were plated with nickel under the same conditions as those disclosed in Example 1 except that sodium tungstate (0.9 g/l), copper citrate (1.4 g/l), and lead chloride (0.65 g/l) were used as desensitizing metal compounds. The principal solution components are shown in Table II. The specimens were thereafter undercoated with vinyl-modified epoxy paint and baked at 275°C for 40 seconds, followed by overcoating with a thermosetting acrylic paint to a total thickness of the coated film of 15 microns and baking at 275°C for 90 seconds. The coated specimens were tested in the same manner as disclosed in Example 1.

Table II shows the results obtained. In the case of lead chloride, the solution was further added with DETA

2Na.2H<sub>2</sub>O (1.35 g/l) in order to enhance the dissolution thereof.

Controls were prepared by plating nickel in the similar manner as disclosed in Controls 1 and 2 except that the coatings were applied under the same conditions as in these examples and tested in the same manner as disclosed in Example 1 to 3. Table II shows also these results for the controls.

TABLE II

| Composition<br>Example | Ni <sup>2+</sup> | Zn <sup>2+</sup> | W <sup>6+</sup> | Cu <sup>2+</sup> | Pb <sup>2+</sup> | O-T Bend<br>Average of<br>5 Panels |
|------------------------|------------------|------------------|-----------------|------------------|------------------|------------------------------------|
| 4                      | 8 <i>all</i>     | 50 <i>all</i>    | 0.5 <i>all</i>  | — <i>all</i>     | — <i>all</i>     | 3.6                                |
| 5                      | 8                | 50               | —               | 0.5              | —                | 3.8                                |
| 6                      | 8                | 50               | —               | —                | 0.5              | 3.6                                |
| Controls 3             | 8                | —                | —               | —                | —                | 4.0                                |
| Controls 4             | 8                | 50               | —               | —                | —                | 1.4                                |

## EXAMPLES 7-9

Specimens were prepared by coating with nickel and coated with the paint and baked under the same conditions as those disclosed in Example 1 except that ammonium meta-vanadate (1.75 g/l) or stannous chloride (0.95 g/l) or copper citrate (1.4 g/l) was used as the desensitizing metal compounds, and all of coating operations were conducted by spraying. Table III shows the results of the adhesion test.

Controls were prepared by plating nickel in the similar manner disclosed in Controls in Examples 1 to 3 except that the coatings were applied under the same conditions as in these examples and tested in the same manner as disclosed in Examples 1 to 3. Table III shows also these results for the controls.

TABLE III

| Composition<br>Example | Ni <sup>2+</sup> | Zn <sup>2+</sup> | V <sup>4+</sup> | Sn <sup>2+</sup> | Cu <sup>2+</sup> | 2-T Bend<br>Average of<br>5 Panels |
|------------------------|------------------|------------------|-----------------|------------------|------------------|------------------------------------|
| 7                      | 8 <i>all</i>     | 50 <i>all</i>    | 0.5 <i>all</i>  | — <i>all</i>     | — <i>all</i>     | 4.8                                |
| 8                      | 8                | 50               | —               | 0.5              | —                | 5.0                                |
| 9                      | 8                | 50               | —               | —                | 0.5              | 4.0                                |
| Control 5              | 8                | —                | —               | —                | —                | 4.6                                |
| Control 6              | 8                | 50               | —               | —                | —                | 2.0                                |

315 prepared by Nihon Parkerizing Co. Ltd.) in a concentration of 20 g/l at 60°C for 3 seconds and any trace of the residual degreasing agent was removed by rinsing with water. Then the specimens were pickled in 5% hydrochloric acid at 25°C for 5 seconds, followed by rinsing with water again. The specimens were then treated with a surface conditioning agent having the following composition at 25°C for 5 seconds. Immedi-

ately after the conditioning, the specimens were treated with a displacement plating solution having the same composition as disclosed in Control 2 at 60°C for 5 seconds. After the plating treatment, any trace of the residual plating solution was removed by rinsing with water. After the treatment with dilute chromic acid (Percolene, Type 62 prepared by Nihon Parkerizing Co. Ltd.) in a concentration of 20 g/l, the specimens were squeezed between rolls to remove any excess of the residual chromic acid and dried with hot air at 105°C. The treatments were all conducted by spraying to complete the nickel plating. The specimens were then coated with a paint under the completely same treating conditions as disclosed in Example 4 to 6. Table IV shows the results obtained on the adhesion test.

TABLE IV

| Composition<br>Example | Sn <sup>2+</sup>                 | W <sup>6+</sup> | Na <sup>+</sup> | Cl <sup>-</sup> | Citric<br>Acid | pH | O-T Bend<br>Average of<br>5 Panels |
|------------------------|----------------------------------|-----------------|-----------------|-----------------|----------------|----|------------------------------------|
| 10                     | 2 <i>all</i>                     | — <i>all</i>    | — <i>all</i>    | 1.3 <i>all</i>  | 19 <i>all</i>  | 2  | 4.0                                |
| 11                     | —                                | 2               | 0.5             | —               | —              | 7  | 4.2                                |
| Control 7              | Without any surface conditioning |                 |                 |                 |                |    | 2.0                                |

## EXAMPLES 10 to 11

These examples show effects obtained in the cases where the article has been pretreated with a solution containing stannous ion or a tungstate as a surface conditioning agent by spraying immediately before the known conventional plating treatment. The stannous ion was added as stannous chloride and the tungsten as sodium tungstate.

Specimens were sampled from non-chromating galvanized steel plate (0.27 × 50 × 100 mm) having a zinc content of 183 grams/m<sup>2</sup>. The specimens were treated in a weak alkaline degreasing agent ("Finecleaner", Type

## EXAMPLE 12

This example shows an embodiment in which specimens were treated with a pickling solution containing ammonium metavanadate prior to the conventional treatment for displacement plating.

Specimens were sampled from non-chromated zinc hot-dip galvanized steel plate (0.27 × 50 × 100 mm) having a zinc content of 183 grams/m<sup>2</sup>. The specimens were treated with a weak alkaline degreasing agent (Finecleaner, Type 135 prepared by Nihon Parkerizing Co. Ltd.) in a concentration of 20 g/l at 60°C for 3 seconds and any trace of the residual degreasing agent

was removed by rinsing with water. They were then pickled in a pickling solution having the following composition at 25°C for 5 seconds, followed by rinsing with water. They were subsequently treated with a displacement plating solution having the same composition as disclosed in Control 2 at 60°C for 5 seconds. After the treatment, they were rinsed with water to remove the residual solution. The specimens were then treated with dilute chromic acid (Percolene, Type 62 prepared by Nihon Parkerizing Co. Ltd.) in a concentration of 20 g/l and they were squeezed between rolls to remove the residual chromic acid and dried with hot air at 105°C. The treatments were all conducted by spraying to complete the nickel coating. The specimens were then coated with a paint under the same painting conditions as disclosed in Example 4 to 6. Table 5 shows the results of adhesion test on the thus-treated surface.

TABLE V

| Composition Example | HCl          | V <sup>4+</sup> | NH <sub>4</sub> <sup>+</sup> | Citric Acid | pH | O-T Bend Average of 5 Panels |
|---------------------|--------------|-----------------|------------------------------|-------------|----|------------------------------|
| 12                  | 10 <i>ml</i> | 1 <i>ml</i>     | 0.2 <i>ml</i>                | 6 <i>ml</i> | 1  | 4.0                          |
| Control 8           | 50           |                 |                              |             |    | 2.0                          |

## EXAMPLE 13

Panels were treated as in Examples 1-3 using 0.3 g/l of antimony added as potassium antimony tartrate as the desensitizer. The adhesion was tested for displacement plating solution having zinc ion contents of 0, 25, and 50 g/l. For comparison, results were also obtained using an antimony-free plating solution.

TABLE VI

| Quantity of Zinc dissolved in the plating solution | 2-T Bend - Average of 5 Panels With Antimony | Control |
|----------------------------------------------------|----------------------------------------------|---------|
| 0 g/l                                              | 5                                            | 4.4     |
| 25 g/l                                             | 4.8                                          | 2.4     |
| 50 g/l                                             | 5                                            | 1.6     |

## EXAMPLE 14

In this example, the adhesion and corrosion resistance were tested for the painted coating on an article treated with a displacement plating solution formulated according to this invention as compared with that of the painted coating on the same type of article pre-treated with a conventional zinc base phosphating solution.

Specimens were sampled from the same hot galvanized steel plate and plated with nickel under the same conditions as disclosed in Example 13 except that potassium antimony tartrate in the displacement plating solution was used in an amount of 0.274 grams (0.1 grams calculated as metallic antimony). Table VII shows results of the adhesion test (conducted in the same manner as in Example 13) and the salt spray test.

Controls were prepared by treating the specimens in an alkaline degreasing agent at 60°C for 10 seconds, followed by rinsing with cold water. The specimens were then pickled with 5% hydrochloric acid for 3 seconds, followed by rinsing with water. The specimens were subsequently treated with a solution containing surface conditioner in a concentration of 3 g/l spraying at 40°C for 3 seconds and then with a zinc base

30 Each test is repeated with 5 specimens and the average reported.

TABLE VII

| Article Prepared According to This Invention | Control treated with Zinc base phosphating Solution |
|----------------------------------------------|-----------------------------------------------------|
| Bend Test                                    |                                                     |
| OT                                           | 4.8                                                 |
| 1T                                           | 5.0                                                 |
| 2T                                           | 5.0                                                 |
| Salt Spray Test (366 hrs.)                   | 0                                                   |
|                                              | 0.5 - 1.0 mm                                        |

## EXAMPLE 15

45 The adhesion of painted film was tested for an article treated with an acidic solution for the displacement plating according to this invention as compared with that for an article treated with a conventional acidic solution for the displacement plating, after aging of both acidic solutions.

50 Specimens were sampled from the same hot galvanized steel plate, plated with iron under the same conditions as disclosed in Example 13 except that the displacement plating solution was replaced by that having the following composition and subjected to the same adhesion test of painted film as disclosed in said example. The results are shown in Table VIII:

|                             |      |                                                     |
|-----------------------------|------|-----------------------------------------------------|
| Ferric oxide                | 15   | grams                                               |
| 35% Hydrochloric acid       | 14.2 | grams                                               |
| 55% Hydrofluoric acid       | 3    | grams                                               |
| Citric acid                 | 5    | grams                                               |
| Potassium antimony tartrate | 0.2  | grams (0.073 grams calculated as metallic antimony) |
| pH                          | 2    |                                                     |

65 Controls were prepared by sampling from the same hot galvanized steel plate and plating with iron under the same conditions as disclosed in the Example except that potassium antimony tartrate was eliminated from the displacement plating solution.

TABLE VIII

| Zn amount dissolved in the plating solution grams/liter | Article pretreated according to this invention | Control |
|---------------------------------------------------------|------------------------------------------------|---------|
| 0                                                       | 3.8                                            | 3.6     |
| 25                                                      | 4.0                                            | 2.0     |
| 50                                                      | 3.8                                            | 2.0     |

## EXAMPLE 16

In this example, the adhesion of painted film was tested for an article in which an antimony compound was added to the solution for a pretreating step, i.e., for the rinsing step with water immediately before the displacement plating step in comparison with that for an article pretreated with a solution containing no antimony compound.

Specimens were sampled from the same hot galvanized steel plate, plated with nickel by employing the same displacement plating solution without any antimony compound as disclosed in Control in Example 13 except that after the pickling and rinsing with water, the surface to be treated was sprayed with an aqueous solution of potassium antimony tartrate in a concentration of 22 g/l (8 g/l calculated as antimony) as a surface conditioner at room temperatures for 5 seconds and coated with a paint. The adhesion test was conducted in the same manner as disclosed hereinbefore. Table IX shows the results obtained.

Controls were prepared by plating with nickel and coated with a paint in the same manner as disclosed in Example 15 except the absence of said surface treatment with the solution containing an antimony compound.

TABLE IX

| Zn amount dissolved in the plating solution grams/liter | Article pretreated According to this Invention | Control treated with zinc base phosphating solution |
|---------------------------------------------------------|------------------------------------------------|-----------------------------------------------------|
| 0                                                       | 4.8                                            | 4.4                                                 |
| 25                                                      | 5.0                                            | 2.4                                                 |
| 50                                                      | 4.8                                            | 1.4                                                 |

50

55

60

65

## EXAMPLE 17

In this example, the adhesion of painted film was tested for an article in which an antimony compound was added to the pickling solution in comparison with that for a substrate pretreated with a conventional pickling solution.

Specimens were sampled from the same hot galvanized steel plate as disclosed hereinbefore, plated with nickel by employing the same displacement plating solution containing no antimony compound as disclosed in Control for Example 13 and coated with a paint in the same manner as disclosed in Example 13 except that the article was sprayed with a pickling solution containing 5 g/l of tartaric acid and 3 g/l of potassium antimony tartrate beside other ingredients at room temperature for 3 seconds. The results obtained are shown in Table X. The table shows also the results of the Control in which the substrate was treated in the same manner as disclosed immediately before except that the pickling solution is replaced by 5% HCl solution.

TABLE X

| Zn content dissolved in the plating solution gram/liter | Article pretreated with pickling solution containing an antimony compound | Control |
|---------------------------------------------------------|---------------------------------------------------------------------------|---------|
| 0                                                       | 4.6                                                                       | 4.4     |
| 25                                                      | 4.8                                                                       | 2.4     |
| 50                                                      | 4.6                                                                       | 1.4     |

What is claimed is:

1. A process for providing a paint base coating on a zinc or zinc alloy surface, comprising contacting said surface with an aqueous acidic composition suitable for the displacement plating of a zinc or zinc alloy surface, consisting essentially of

- a soluble heavy metal compound selected from the group consisting of nickel, cobalt and iron in an amount of 0.1 - 50 g/l expressed as the heavy metal; and
- a soluble compound of a desensitizing metal selected from the group consisting of antimony, tin, copper, lead, germanium, vanadium, arsenic and tungsten in an amount of at least 0.001 g/l expressed as the metal.

2. The process of claim 1 wherein said contact is effected by the immersion or spray technique.

\* \* \* \* \*